

## UNITED STATES PATENT OFFICE

HENRY L. COLES, OF HAMILTON, OHIO, ASSIGNOR TO GUARDIAN METALS COMPANY, OF HAMILTON, OHIO, A CORPORATION OF DELAWARE

## PROCESS FOR PRODUCING COMPOSITE METALS

No Drawing. Original application filed November 22, 1927, Serial No. 234,957. Divided and this application filed November 9, 1928. Serial No. 318,313.

This application is a division of my application, Serial No. 234,957, filed November 22, 1927, for "composite metals and process for producing the same".

5 This invention relates to an improved process for fabricating composite metal plates and the like. In my application above referred to, there has been described a process for fabricating composite metal plates, 10 and more particularly the improved product resulting from such process. In the present case, in order to secure intimate contact between the metal of the core and of the sheath to form a composite or compound metal 15 plate, the core members are first subjected to a preliminary treatment.

In this treatment the metallic core is sand-blasted or otherwise treated to remove surface matter such as oxides and the like, after 20 which it is sprayed with a concentrated solution of a nitrogenous material such as alkali nitrite, my preferred composition being sodium nitrite ( $\text{NaNO}_2$ ). The function of the sodium nitrite is to improve the wetting qualities 25 of the core metal and adapt it to be wetted by the molten sheathing material or metal such as copper or the like. Usually after spraying, heat is applied by a torch to dry the core, care being taken to restrict the 30 amount of heat to that necessary for drying, without effecting any substantial decomposition of the sodium nitrite. The result of this treatment is a metallic core intimately coated with a layer of the sodium nitrite. When 35 molten metal, such as copper, is cast in and around such a core member, it decomposes the sodium nitrite, liberating quantities of gases such as nitrogen which serve to force out the air from the mold chamber and to 40 provide substantially oxygen-free atmosphere therein. This freedom from oxygen prevents the formation of the noxious oxides of copper, and with these oxides absent, the unalloyed character of a highly refined 45 sheath metal may be preserved.

A particular example of the improved results to be procured by the application of the present process is in the casting of compound metal bodies for use in the manufacture 50 of burglar-proof safes and vaults, as

exemplified in my present application, above noted, in which a metallic core of drill-proof metal composition or alloy, of the types disclosed in my co-pending applications, Serial Nos. 730,194 and 86,034, (in which the compositions include preponderating amounts of tungsten with minor amounts of molybdenum, carbon or copper, or ferrous alloys having a high percentage of chromium and manganese) is formed into any desired configuration, and intimately coated with a concentrated solution of sodium nitrite. These so-treated bodies are then placed in a mold, or they may be preliminarily placed in a mold and the nitrite solution applied by spraying, after which a suitable sheathing metal such as copper is poured into the mold.

During the casting operation the molten metal is preferably poured as slowly as is consistent with results to be obtained. The primary consideration is that the molten metal shall contact with the core metal at such a rate of speed as will insure an adequate preheating thereof without chilling the pour. This preheating also serves to decompose the nitrite coating, setting free gaseous nitrogen and its oxides, which, as has already been pointed out, sweep out the air from above the surface of the advancing metal.

The alkali molecules set free by the decomposition of the nitrite unite with any siliceous impurities present, and form a free-flowing slag coating over the surface of the pour, thereby adding an additional protective agent to co-act with the gaseous blanket previously described. The thorough cleaning which the surface of the core metal undergoes, as a result of this treatment, greatly enhances the wetting capacity of the molten metal by assuring an absolutely clean metal to metal surface. The advancing metal flows into and through the interstitial spaces between the slats of which the core is preferably formed, forming a substantially continuous sheath therearound; and being in intimate contact therewith, the result is essentially a composite metal plate comprising a hard core of drill-resistant metal and an outer protecting sheath of ductile and com-

pressible metal such as copper which offers a high degree of heat conductivity.

It has been found that in addition to a mere wetting of the core metal by the sheath metal, there results a true combination or alloying between them which is considerably greater than a strict welded union. The depth of this union or "case" as it is known in the art, is determined by the temperature and time of contact, and as the mould is preferably cooled very slowly, the reaction proceeds over a maximum period. The mutual solution of the constituents of the several alloys proceeds under optimum conditions, and the core and sheath are joined in a substantial mono-metallic structure.

The process herein described is adapted for a wide variety of metallurgical purposes, and more particularly for the casting of non-ferrous metals generally, which are readily oxidized in their molten condition. The ease of decomposition of this material, sodium nitrite, is of particular importance in the present invention, as it affords a ready means of providing a non-oxidizing atmosphere in casting molds and the like without involving the necessity of using gaseous nitrogen, or other non-oxidizing gases with the attendant trouble of the apparatus required.

By way of résumé it will be noted that by merely coating the mold walls with a concentrated solution of sodium nitrite, or any other suitable compound, such as the other alkali nitrites, the molten metal in contact with the mold walls readily decomposes the alkali nitrites, copious volumes of nitrogen gas is set free and acts to sweep, or force out any air present from the mold chamber. In addition, the alkali residues set free by the liberation of the nitrogen component react with any siliceous material present to form a free-flowing slag which covers the top of the advancing metal, thus co-operating with the non-oxidizing gaseous blanket to prevent any contact between the metal and the outside air. Where core members of non-ferrous metal are used, the cores are previously coated with the concentrated nitrite solution, and due to the vigorous chemical action between the constituents of the nitrite compound and any non-metallic impurities which may be present on the surface of the core under the influence of the molten metal, the core surface is thoroughly cleansed and presented to the advancing metal, not only in a condition wherein it is free from occluded oxygen and the like, but also in which it is particularly adapted to combine or alloy with the sheath metal, where such alloying is possible.

It will now be appreciated that there has been provided an improved process for the production of composite metal castings, this process being characterized by the discovery that the presence of an alkali nitrite in the mold, or applied to a core member in a mold,

enables the ready preparation of difficult castings without involving any great expense in special machinery required for gaseous deoxidants of like blanketing materials.

What is claimed is:

1. A method of producing compound metallic plates, comprising coating a core member with a readily decomposable nitrogenous compound, and casting a sheath of metal in and around the core. 70

2. A method of producing compound metallic plates, comprising coating a core member with an alkali nitrite, and casting a sheath of metal around the core. 75

3. A method of producing compound metallic plates, comprising coating an apertured core member with sodium nitrite and casting a sheath of metal in and around the core. 80

4. A method of producing compound metallic structures, comprising coating an apertured core member with sodium nitrite, casting a sheath of metal around the core under determined conditions of temperature and rate of pour, whereby to assure optimum conditions of reaction. 90

5. A method of producing burglar-proof safes, comprising forming a drill-proof core member, spraying the core with sodium nitrite, and casting a heat-conductive metal in and around the core. 95

6. A method of producing burglar-proof vault doors, comprising forming a drill-proof core member, spraying the core with an alkali nitrite, and casting a sheath of heat-conductive metal in and around the core. 100

7. A method of producing compound metallic plates, comprising casting a sheath of metal around a metal core member in the presence of nitrogen liberated in situ. 105

8. A method of producing compound metallic plates, comprising casting a sheath of metal around a metal core member in the presence of nascent nitrogen. 110

9. In the production of metallic compound plates having an inner core member and an external sheath cast therearound, the improvement which comprises simultaneously cleansing the surface of the core member and forming a non-oxidizing protective atmosphere about the said core by reacting the molten sheath metal with a compound adapted to liberate nitrogen gas and an alkali residue. 115

10. In the production of compound metallic plates having an inner core member and an external sheath cast therearound, the improvement which comprises simultaneously forming a protective slag on the surface of the molten sheath metal and an atmosphere of inert gas around the said core. 120

11. The method of forming compound metal plates from readily oxidizable metals, comprising positioning a metal core member in a mold, coating the core and the walls of 125

the mold with a nitrogenous compound adapted to liberate nitrogen gas and a slag-forming residue when strongly heated, and flowing a molten sheath of metal into said mold and around said core, whereby to form an atmosphere of nitrogen gas in the mold chamber and a free-flowing slag coating on the said flowing molten metal.

5 This specification signed this 8th day of  
10 November, 1928.

HENRY L. COLES.

15

20

25

30

35

40

45

50

55

60

65